

Patented Mar. 26, 1929.

1,706,717

## UNITED STATES PATENT OFFICE.

ALBERT WAGNER, OF GROSS-ZSCHACHWITZ, NEAR DRESDEN, GERMANY, ASSIGNOR TO  
THE FIRM FR. KUTTNER, OF PIRNA, SAXONY, GERMANY.

### PROCESS OF PRODUCING FINE FIBER ARTIFICIAL SILK.

No Drawing. Application filed March 25, 1927, Serial No. 178,507, and in Germany June 11, 1926.

The production of fine fiber artificial silk from a solution of ammoniated copper oxide cellulose according to the well known stretch spinning process has hitherto been effected by treating the spun silk, for which water was used as stretching medium, after passing out from the spinning funnel in a 12% water solution of sulphuric acid, as a result of which cellulose hydrate is produced. The 10 thus hardened silk has a comparatively small degree of elasticity and plasticity.

The cellulose fiber containing copper in wet condition is more plastic than that containing no copper or but very little. It has therefore already been suggested to carry out the hardening process so that even when using sulphuric acid as a precipitating medium, the fiber will still retain its copper. It is, however, technically difficult to carry 20 out this method so that the thread will retain the copper and only lose the ammonia which acts as a solvent and produces stickiness.

By employing a well known process with 25 iron sulphate, it is possible to produce a cellulose fiber containing copper whose individual threads will not stick together. The employment of iron sulphate because of the separation of ammonia produces self oxidizing iron hydrate which when freed from copper is objectionable.

I have found that a water solution of 30 aluminum sulphate can be advantageously used as a hardening medium. The fiber derived from such a bath contains in addition to copper, residues of sulphuric acid and aluminum. About half of the whole fiber

consists of cellulose. The effect of this method is that the individual threads easily separate from one another and that a green 40 copper cellulose fiber is produced which when wet is plastic to the highest degree, so that a silk is produced which is very expansible. The plasticity of the wet fiber containing copper is so high that even when 45 finished the fiber can be stretched on different rollers without reducing its expansibility when dry.

After the fiber has been treated with aluminum sulphate it is wound around spools 50 or the like, washed in water to free it from salts soluble in water. Thereupon the fiber is freed from copper by sulphuric acid, again washed, soaped and dried. Inorganic acids such as sulphuric acid or the like may 55 be added to the aluminum sulphate in order to dissolve the aluminum hydrate not absorbed by the fiber.

The bath, either cold or warm, is advantageously made up of a 12% water solution 60 of aluminum sulphate.

What I claim is:—

A process of producing fine fiber artificial silk, consisting in first forming strands from a solution of ammoniated copper oxide cellulose according to the stretch spinning method, then treating said strands in a bath containing a solution of aluminum sulphate, then winding said strands on spools or the like, then washing them, then treating the 65 same in sulphuric acid, then again washing and finally drying.

In testimony whereof I affix my signature.

ALBERT WAGNER.